

(No Model.)

C. J. EAMES.

FURNACE FOR THE MANUFACTURE OF SPONGE, WROUGHT IRON, AND  
STEELY IRON DIRECT FROM THE ORE.

No. 318,608.

Patented May 26, 1885.

Fig. 1.



Fig. 2.



Fig. 3.



Witnesses -

G. A. Tauberschmitt  
H. A. Moulton

Inventor

Charles J. Eames  
by F. W. Ritter Jr  
Attest

# UNITED STATES PATENT OFFICE.

CHARLES J. EAMES, OF NEW YORK, N. Y., ASSIGNOR TO THE CARBON IRON COMPANY, OF SAME PLACE.

FURNACE FOR THE MANUFACTURE OF SPONGE, WROUGHT-IRON, AND STEELY IRON DIRECT FROM THE ORE.

SPECIFICATION forming part of Letters Patent No. 318,603, dated May 26, 1885.

Application filed February 27, 1885. (No model.)

*To all whom it may concern:*

Be it known that I, CHARLES J. EAMES, a citizen of the United States, residing at New York city, in the State of New York, have invented certain new and useful Improvements in Reduction of Iron Ore in the Furnaces for the Manufacture of Sponge, Wrought-Iron, and Steely Iron Direct from the Ore; and I hereby declare the following to be a full, clear, and exact description of the same, reference being had to the accompanying drawings, in which—

Figure 1 is a longitudinal vertical section of a furnace embodying my invention. Fig. 2 is a horizontal section of the rear end of the furnace on the line  $yy$ , Fig. 3; and Fig. 3 is a vertical transverse section on the line  $xx$ , Fig. 1.

Like letters refer to like parts wherever they occur.

My present invention relates to the construction and arrangement of a deoxidizing and carburizing furnace so that a continuous process can be conducted therein, whereby several material advantages are obtained over present furnaces and methods. For instance, first, a preparatory or drying and heating chamber for the ore and carbon is provided, wherein all moisture is expelled and a preliminary heating of the matter to be treated takes place; secondly, the deoxidizing and carburizing hearth or chamber is so placed at the rear of the furnace and at the discharge end of the drying or preparatory chamber as to be uniformly heated and the heat thereof maintained without variation; and, thirdly, a balling-hearth is provided and so arranged with relation to the deoxidizing and carburizing hearth as to receive the charge deoxidized therefrom, and thus enables the furnace to be worked continuously.

The balling-hearth may be of the usual silicious character. The deoxidizing-hearth will be covered with a friable graphitic covering, either in compact form or in the form of lumps, as desired.

I will now proceed to describe my invention more specifically, so that others skilled in the art to which it appertains may apply the same.

In the drawings, A A indicate brick arches supporting the sole or plate B of a furnace, which shall be about double the length as well as double the width of ordinary reverberatory

furnaces. At one end of this furnace is the usual or any approved fire-chamber, a, having an ash-pit, b, closed by the door c. Into this ash-pit a blast-pipe, d, delivers. There is the usual fire-bridge, e, back of which and parallel therewith is the transverse bridge f, which divides the chamber into a balling-hearth, C, located in direct proximity to the fire-chamber, where the highest heats prevail, and a deoxidizing and carburizing chamber, D, distant from the fire-chamber a, or where a lower dull-red or deoxidizing temperature prevails.

The balling-hearth C may have the usual sand bottom, or any approved fettling used in like chambers; but the deoxidizing and carburizing hearth D is covered for a depth of four to six inches with a friable graphitic bottom, (such as forms the subject-matter of Serial No. 144,152, filed September 27, 1884,) or with friable graphitic lumps l, (such as form the subject-matter of Serial No. 149,823,) consisting of small lumps of the "graphitic carbon" of commerce, such as is obtained at Cranston, Rhode Island, and elsewhere, and just as it comes from the mine. This deoxidizing-hearth D may, if desired, be divided longitudinally by a slight bridge, h, (part of which is shown in Fig. 2,) the purpose of which, when used, will hereinafter appear.

$a'$ ,  $c'$ , and  $d'$  indicate working doors for the fire-chamber and hearths.

Supported on and projecting into the rear end of the furnace is a vertical feeding and drying chamber, E, which is by preference a cylindrical fire-brick stack some ten or twelve feet (more or less) in height, and of suitable diameter—say fifteen inches to two feet—having an opening or door,  $e'$ , below, through which it discharges or feeds down on the deoxidizing and carburizing hearth. This feeding and drying chamber is encompassed at its base by the flues  $w$ , by which the waste gases, &c., escape to a flue, W, leading to a stack beneath a boiler, or to other desired point.

S S indicate dampers which may be inserted in the flues  $w$ , if in the working of the furnace it becomes necessary or desirable to change the draft from one to the other side of the hearth D.

The above is a general description of a form of furnace which I have found very effective

for the purposes hereinbefore set forth, and which may be varied in detail without departing from the spirit of my invention, provided the characteristic features and relative arrangement of the chambers are preserved.

The devices, being of the general character hereinbefore set forth, will be operated as follows: The deoxidizing and carburizing agent employed, which, though not necessarily, is 10 preferably friable graphitic lumps—such as the graphitic carbon of commerce, hereinbefore referred to—is intermingled with the ore which is to form the charge. As a matter of general direction, I will say that I have found 15 twenty per cent. of such graphitic carbon to eighty per cent. of ore sufficient. The charge of ore and deoxidizing agent, which generally contains more or less moisture, is then charged into the drying and feeding chamber E, and 20 therein is subjected to the transmitted heat from the furnace for several hours, or during the deoxidation of the previous charge. The waste products from the furnace pass around the base of this chamber E through the waste-flues *w w* and into the main flue W. So far as I am aware none of the waste products pass 25 through the charge in the drying and feeding chambers. From the drying and feeding chambers the charge, properly dried and heated, is 30 drawn down upon the graphitic hearth of the deoxidizing and carburizing chamber D, is spread out so as to be fully subjected to the currents of heated gases, &c., and is retained on said hearth until deoxidation, or deoxidation 35 and the required carburization, is completed. When this is accomplished, the charge is drawn in small masses or in bulk over the bridge-wall *f* onto the balling-hearth C, where it is subjected to a higher temperature, sufficiently high to cause the agglomeration of the mass, and is balled in the usual manner and removed to the blooming apparatus.

The above is a general statement of the manner in which the furnace is worked; but 45 in practice it will be noted that after the first charge in chamber E is ready to be drawn on the deoxidizing-hearth D the working of the furnace will become continuous, as the ore and carbon composing the charge can be fed 50 into the chamber E from time to time as it sinks therein. The charge for the deoxidizing and carburizing hearth D can be drawn first on one side of the hearth (or bridge-wall *h*, if such is used,) and then on the other, and from 55 hearth D the deoxidized and carburized ore or sponge can be drawn onto the balling-hearth C in like order.

In practice I have found that the first charge in chamber E can be prepared for the deoxidizing-hearth in four (4) or five (5) hours, and thereafter the necessary amount of ore and graphitic lumps added to the top of the charge in chamber E will be fully prepared by the time it reaches the discharge-door *e*. 60

The ore, &c., as it comes from the chamber E, will require about an hour for treatment on the hearth D, and then can be transferred to 65

the balling-hearth C, where it can be balled, ready for removal in from twenty minutes to half an hour, so that the furnace is practically 70 continuous in its operation.

It is to be noted that the fire in chamber *a* should be kept in such condition that the temperature on hearth D will be about a dull red, and this will always insure the proper 75 temperature on the balling-hearth C.

If sponge only is wanted, it is drawn as soon as deoxidation is complete, without transferring it to the balling-hearth; but if wrought-iron is desired it is transferred to the balling-hearth C, and thence to the blooming apparatus; while if steel or steely iron is desired the ore, after it is deoxidized or becomes sponge, is retained in the hearth D a further time proportionate to the degree of carburization required, after which it is transferred to the balling-hearth C, and thence to the blooming apparatus, as before specified.

The advantages of my invention are the simplicity of the devices, the continuous 90 character of the operations capable of being conducted therein, and the great reduction of time required in the several steps of the process.

Having thus described my invention, what 95 I claim, and desire to secure by Letters Patent, is—

1. A deoxidizing-furnace for the treatment of ores, said furnace having a balling-hearth and a deoxidizing-hearth provided with a 100 friable graphitic bottom, said hearths arranged in sequence, substantially as and for the purposes specified.

2. The combination, in a furnace for deoxidizing ores, of a feeding and drying chamber 105 for preliminary treatment of the charge, and a deoxidizing-hearth having a friable graphitic bottom, substantially as and for the purposes specified.

3. In a furnace for deoxidizing ores, the 110 combination of a balling-hearth, a deoxidizing-hearth having a friable graphitic bottom, and a preliminary drying and feed chamber for receiving the fresh charge, all arranged in sequence, substantially as and for the purposes 115 specified.

4. In a furnace for deoxidizing ores, the combination of a balling-hearth and a deoxidizing-hearth having a longitudinal bridge-wall, substantially as and for the purposes 120 specified.

5. In a furnace for deoxidizing ores, the combination of a drying and feeding chamber, a deoxidizing-hearth having a longitudinal bridge-wall, and a balling-hearth, all arranged 125 in sequence, substantially as and for the purposes specified.

In testimony whereof I affix my signature, in presence of two witnesses, this 27th day of February, 1885.

CHARLES J. EAMES.

Witnesses:

F. W. RITTER, Jr.,  
G. A. TAUBERSCHMIDT.